

## 1

3,694,214

### LIGHT-SENSITIVE COLOR-PHOTOGRAPHIC EMULSIONS

Masakumi Iwama, Isaburo Inoue, Teruo Hanzawa, Kenro Sakamoto, and Takaya Endo, Tokyo, Japan, assignors to Komishiroku Photo Industry Co., Ltd.  
No Drawing. Continuation-in-part of abandoned application Ser. No. 778,774, Nov. 25, 1968. This application Oct. 14, 1970, Ser. No. 80,749

Int. Cl. G03c 1/40

U.S. Cl. 96—100

7 Claims

#### ABSTRACT OF THE DISCLOSURE

A light-sensitive color photographic silver halide emulsion which comprises a coupler of the general formula



wherein

$R_1$  represents an aliphatic hydrocarbon radical having 8–20 carbon atoms,

$R_2$  represents hydrogen or a lower alkyl group,

$B$  represents yellow or magenta coupler residue,

$X$  represents a radical connecting  $B$  and



$n$  is 0 or 1.

This application is a continuation-in-part of application Ser. No. 778,774, filed Nov. 25, 1968, now abandoned.

This invention relates to a light-sensitive silver halide color-photographic emulsion. More particularly, the present invention relates to a light-sensitive silver halide color-photographic emulsion containing, as a protected coupler or alkali-soluble coupler, a novel coupler compound of the general formula



wherein  $R_1$  is an aliphatic hydrocarbon radical of 8 to 20 carbon atoms;  $R_2$  is hydrogen or a lower alkyl radical;  $B$  is a radical which couples with the oxidation product formed during color development to form a yellow or magenta color;  $X$  is a group capable of bonding the  $B$  group with a group of



and  $n$  is 0 or 1.

In order to be usable for commercial purposes, a protected coupler is required, in general, to satisfy the following conditions:

(1) The coupler should be prepared in high purity according to a simple synthetic process from readily available inexpensive materials.

(2) The coupler and a dye formed by color development should be well soluble in a high boiling solvent, such as tricresyl phosphate, dibutyl phthalate, etc., to give a high concentration solution.

(3) The coupler should have no detrimental effects, such as fogging, desensitization, etc., on a silver halide emulsion.

## 2

(4) When the dispersion of the coupler in a silver halide emulsion is coated and dried on a support, the coupler should give a stable photographic layer which has not suffered from crystallization.

(5) The coupler should be favorable in color developing property, be excellent in spectral absorption characteristic of the resulting color-developed dye image and be fast to heat, light and humidity, and it should not cause staining of the unexposed area.

With an aim to satisfy the above requirements, many studies have been made and various couplers have been proposed hitherto. However, there has not been found a coupler which can satisfy the above requirements.

For example, the coupler disclosed in U.S. Pat. 2,875,057 which is represented by the formula



is excellent in solubility for high boiling solvents, but is extremely expensive. Further it is likely to be crystallized out at its concentrated state.

The known coupler disclosed in Japanese patent publication No. 2,837/1964, which is represented by the formula



is much more improved in solubility for high boiling solvents than the coupler of U.S. Pat. 2,875,057 but is very expensive because the lipophilic component thereof should be synthesized through several steps.

On the other hand, an alkali-soluble coupler also is required to satisfy, in addition to the before-mentioned requirements (1) to (5), with the good dissolution in aqueous alkali and the ready dispersion in photographic emulsions. In spite of keen studies in the prior art, there have never been found alkali-soluble couplers fully satisfactory to the above requirements.

For example, long chain alkyl succino-monoamide couplers disclosed in Japanese patent publication Nos. 18,735/64 and 12,836/66 can form a dye image excellent in light, humidity and heat fastness, but it is likely to be crystallized out from the emulsion or photographic coating due to its poor alkali solubility, thereby adversely affecting on transparency of unexposed area and colored dye image.

$\alpha$ -Sulfonated long chain fatty acid amide couplers disclosed in U.S. Pat. 2,829,975 and Japanese patent publication No. 18,333/63 is excellent in alkali solubility, is readily dispersible or miscible in emulsions and has little tendency to crystallize out. However, these couplers usually are very difficult in preparation and purification.

We have now found that a coupler of the aforementioned general formula is very useful as either of a

protected coupler and an alkali-soluble coupler. The compounds used as couplers in the present invention can be easily prepared in a simple way by using long chain alkyl bromide and malonic acid ester as starting materials which are inexpensive and readily available. A light-sensitive color-photographic material which comprises a support and, coated thereon, a layer of the emulsion of the present invention can yield, through exposure to light and subsequent color development according to a usual method, a clear dye image with high color density. Transparency at unexposed area also is excellent. Further, the said color-photographic material is entirely free from fogging, desensitization and any other adverse effects on photographic properties.

When a compound of the aforementioned general formula is used as a protected coupler, a coupler dispersion having the high ratio of the coupler to the solvent amount is obtained because of high solubility of

the coupler in dibutyl phthalate, tricresyl phosphate, etc. Further, a photographic layer obtained from the said dispersion is stable and does not suffer from the crystallization of the said coupler.

When a compound of the aforementioned general formula is used as an alkali-soluble coupler, it can show better solubility than the known long chain alkyl succinmonoamide coupler. The compound is readily miscible or dispersible in photographic emulsion and does not cause crystallization.

10 The remarkable improvement of a light-sensitive color-photographic emulsion according to the present color-photographic emulsion according to the present invention may be considered due to the existence of a carboxyl or lower alkoxy-carbonyl group at the  $\alpha$ -position of a long chain fatty acid amide structure.

15 Now typical coupler compounds useful in the invention are listed hereunder.

|                                                                                     | M.P. (°C.) |
|-------------------------------------------------------------------------------------|------------|
| (1)-----                                                                            | 77-78      |
|   |            |
| (2)-----                                                                            | 67-69      |
|   |            |
| (3)-----                                                                            | 180-181    |
|  |            |
| (4)-----                                                                            | 93-96      |
|  |            |
| (5)-----                                                                            | 160-161    |
|  |            |
| (6)-----                                                                            | 68-69      |
|  |            |
| (7)-----                                                                            | 267-269    |
|  |            |

M.P. (° C.)

|           |  |         |
|-----------|--|---------|
| (8)-----  |  | 272-274 |
| (9)-----  |  | 48-49   |
| (10)----- |  | 107-108 |
| (11)----- |  | 117-118 |
| (12)----- |  | 207-209 |
| (13)----- |  | 244-245 |

Couplers usable in this invention are synthesized by the following method:

Diethyl alkylmalonate obtained by the reaction of a long-chain alkyl bromide with diethyl malonate is hydrolysed to the mono-ester and treated with thionyl chloride. The resulting acid chloride is condensed with an appropriate coupler intermediate having amino group to give an yellow or magenta coupler used in this invention.

#### PREPARATIVE EXAMPLE 1

##### Synthesis of diethyl n-hexadecylmalonate

Into a 2 l. three-necked flask was charged a solution of 24.2 g. of metallic sodium in 480 ml. of ethyl alcohol, and 160 g. of diethyl malonate was added thereto. The mixture was stirred at 60°-70° C. for 15 minutes. 336 g. of diethyl malonate was added to the mixture under

boiling, and the mixture was boiled with reflux for additional 2 hours. Thereafter, 450 ml. of the ethyl alcohol was removed by distillation, and the distillate was charged with water to separate an oil. The oil thus separated was extracted with ether. The ethereal solution was washed with water, dried and then distilled to remove the ether. The residue was distilled under reduced pressure to obtain 250 g. (yield: 65%) of a fraction having a boiling point of 182°–185° C. at 0.05 mm. Hg.

5 an ion exchange resin, Amberlite G 120, and then a column with Amberlite G 400. The solvent was removed by distillation under reduced pressure, and the residue was recrystallized from 500 ml. of n-hexane, whereby 30 g. (yield 51%) of pale yellow powder having a melting point of 77°–78° C.

5 The exemplified couplers 1, 2, 5, 6, and 10 are those which have been prepared by using intermediates and acylating agents set forth in Table 1.

TABLE 1

| Coupler | Intermediate                                                     | Acylation agent                               | Melting point of coupler (°C.) | Nitrogen content (percent) | Cal'd | Found |
|---------|------------------------------------------------------------------|-----------------------------------------------|--------------------------------|----------------------------|-------|-------|
| 1       | $\alpha$ -(4-aminobenzoyl)-5-ethoxycarbonyl-2-methoxyacetanilide | $\alpha$ -Ethoxycarbonylmystic acid chloride  | 77–78                          | 4.74                       | 4.71  |       |
| 2       | $\alpha$ -(4-aminobenzoyl)-2-methoxyacetanilide                  | $\alpha$ -Ethoxycarbonylstearyl acid chloride | 67–69                          | 4.50                       | 4.20  |       |
| 5       | 4-aminobenzoylacetanitrile                                       | $\alpha$ -Ethoxycarbonylcapric acid chloride  | 93–96                          | 7.25                       | 7.30  |       |
| 6       | 3-(4-aminophenyl)-pyrazolinobenzimidazole                        | $\alpha$ -Ethoxycarbonylmystic acid chloride  | 160–161                        | 10.56                      | 10.30 |       |
| 10      | 1-(2,4,6-trichlorophenyl)-3-(3-aminobenzamide)-5-pyrazolone      | $\alpha$ -Ethoxycarbonylstearyl acid chloride | 48–49                          | 7.61                       | 7.43  |       |

Elementary analysis.—Calc. (percent): C, 71.83; H, 11.53. Found (percent): C, 71.64; H, 11.85.

#### PREPARATIVE EXAMPLE 2

##### Synthesis of monoethyl n-hexadecylmalonate

A mixture comprising 200 g. of the diethyl ester obtained by Preparative Example 1 and a solution of 29.5 g. of potassium hydroxide in 610 ml. of ethyl alcohol was boiled for 5 hours. The alcohol was then removed by distillation, and the distillate was charged with 600 ml. of water and 50 ml. of concentrated hydrochloric acid. The precipitate formed was collected by filtration, washed with water, dried and recrystallized from n-hexane. There was obtained 165 g. (87%) of white powder having a melting point of 43°–44° C.

Elementary analysis.—Calc. (percent): C, 70.74; H, 11.31. Found (percent): C, 70.72; H, 11.56.

#### PREPARATIVE EXAMPLE 3

##### Synthesis of $\alpha$ -ethoxycarbonylstearyl acid chloride

72 grams of the monoethyl ester synthesized according to Preparative Example 2 was mixed with 71 g. of thionyl chloride, and the mixture was allowed to stand at ordinary temperature overnight. The thionyl chloride was then distilled under reduced pressure, and the distillate was used in the step of acylation which follows.

Using n-octylbromide or n-dodecylbromide in place of the n-hexadecylbromide and following the procedures of Preparative Examples 1 and 2, there were prepared long chain alkyl malonates having 8 and 12 carbon atoms, respectively, which were then converted to corresponding acid chlorides according to the procedure of Preparative Example 3.

| Alkyl group                       | Diester           |                 | Monoester  |                 |
|-----------------------------------|-------------------|-----------------|------------|-----------------|
|                                   | B.P. (°C./mm. Hg) | Yield (percent) | M.P. (°C.) | Yield (percent) |
| n-C <sub>8</sub> H <sub>17</sub>  | 939–141/3.0       | 65              | (1)        | 93              |
| n-C <sub>12</sub> H <sub>25</sub> | 168–169/2.0       | 60              | 33–34      | 92              |

(1) Oily product.

#### PREPARATIVE EXAMPLE 4

##### Synthesis of $\alpha$ -(4- $\alpha$ -ethoxycarbonyl-myristoylaminobenzoyl)-5-ethoxycarbonyl-2-methoxy-acetamide (exemplified coupler 1)

To a mixture comprising 36 g. of  $\alpha$ -(4-aminobenzoyl)-5-ethoxycarbonyl-2-methoxyacetanilide and 150 ml. of pyridine was added 33 g. of  $\alpha$ -ethoxycarbonylmystic acid chloride, and the mixture was heated at 90°–95° C. for 1 hour. The reaction mixture was diluted with water to separate an oily product. The oily product was extracted with ethyl acetate, washed with water and dried. The ethyl acetate was removed by distillation, and the residual oily product was dissolved in methyl alcohol and the solution was passed through a column packed with

#### PREPARATIVE EXAMPLE 5

##### Synthesis of 1-(4-carboxyphenyl)-3-(4- $\alpha$ -carboxystearoylaminobenzamide)-5-pyrazolone (exemplified coupler 9)

25 36 grams of 1-(4-ethoxycarbonylphenyl)-3-(4- $\alpha$ -ethoxycarbostearoylaminobenzamide) - 5 - pyrazolone (M.P. 162°–163° C.) was added to a mixture comprising 172 ml. of ethyl alcohol and 86 ml. of 20 w/w. percent of aqueous sodium hydroxide solution, and the resulting mixture was stirred at 45°–50° C. for 10 minutes. The mixture was diluted with 500 ml. of water and acidified with hydrochloric acid. The precipitate deposited was collected by filtration, washed with water and dried. The dried precipitate was dissolved in 100 ml. of dimethylformamide and diluted with methyl alcohol to deposit a coupler. The dilution was left to stand overnight, and the coupler was collected by filtration, washed with methyl alcohol and dried. White powder having a decomposition temperature of 283°–284° C. was obtained. The yield was 25 g. (77%).

40 Elementary analysis.—Calc. (percent): N, 8.64. Found (percent): N, 8.50.

The exemplified couplers 4, 7, 8, 11, 12 and 13 are prepared respectively from starting materials set forth in Table 2 in accordance with the procedure of Preparative Example 5.

45

TABLE 2

| Coupler | Starting material                                                                                  | Melting point of coupler (°C.) |       |      | Nitrogen content (percent) |  |
|---------|----------------------------------------------------------------------------------------------------|--------------------------------|-------|------|----------------------------|--|
|         |                                                                                                    | Cal'd                          | Found |      |                            |  |
| 50      |                                                                                                    |                                |       |      |                            |  |
| 4       | $\alpha$ -[3-( $\alpha$ -ethoxycarbonylstearyl-amino)benzoyl]-5-carboxy-2-methoxyacetanilide.      | 180–181                        | 4.20  | 4.49 |                            |  |
| 7       | 1-phenyl-3- $\alpha$ -ethoxycarbonylstearylaminopyrazolone.                                        | 68–69                          | 8.65  | 8.25 |                            |  |
| 55      | 8 1-[4-(4-tertiarybutyl)phenoxyl]-3-sulfophenyl-3- $\alpha$ -ethoxycarbonylstearylaminopyrazolone. | 267–269                        | 5.74  | 5.56 |                            |  |
| 11      | 1-(2,4,6-trichlorophenyl)-3-[3-( $\alpha$ -ethoxycarbonylstearylaminobenzyl)-5-pyrazolone.         | 107–108                        | 7.91  | 7.69 |                            |  |
| 12      | 1-(2,4,6-trichlorophenyl)-3-[4-( $\alpha$ -ethoxycarbonylstearylaminophenyl)-5-pyrazolone.         | 117–118                        | 7.57  | 7.40 |                            |  |
| 60      | 13 6- $\alpha$ -ethoxycarbonylstearylaminodiazolone.                                               | 207–209                        | 9.14  | 9.05 |                            |  |

#### PREPARATIVE EXAMPLE 6

65 5 Synthesis of 1-(4-carboxyphenyl)-3-(4- $\alpha$ -carboxystearoylaminobenzamide) - 4-(4-methoxyphenylazo)-5-pyrazolone (exemplified coupler 14)

70 10.0 grams of p-anisidine was diazotized with 120 ml. of water, 30 ml. of concentrated hydrochloric acid and 8.0 g. of sodium nitrite, and 400 ml. of ethyl alcohol was added thereto.

To a solution of 32.4 g. of the exemplified coupler 9 in 324 ml. of pyridine was added at 5°–10° C. the solution of diazonium salt prepared above. The mixture was stirred

for 3 hours and then diluted with water and charged with 400 ml. of hydrochloric acid. The precipitate deposited was collected by filtration, washed with water and dried.

The precipitate thus obtained was dissolved in 100 ml. of dimethylformamide and diluted with methyl alcohol, whereby an orange precipitate was deposited. The precipitate was collected by filtration, washed with methyl alcohol and dried to obtain orange powder having a melting point of 244°-245° C. The yield was 14.0 g. (36%).

*Elementary analysis.*—Calc. (percent): N, 10.73. Found (percent): N, 10.51.

In the application of these couplers as protected couplers, a coupler is dissolved in a high boiling solvent such as tricresyl phosphate, dibutyl phthalate, etc. alone or, if necessary, in a mixture of the high boiling solvent with a low boiling solvent such as ethyl acetate, butyl acetate, butyl propionate, etc. The resulting solution is dispersed in an aqueous gelatin solution containing a surfactant by passing the mixture through a high speed rotary mixer or colloid mill. The resulting dispersion is added to a silver halide photographic emulsion and the thus treated emulsion is coated on a support such as film base, baryta paper, etc. and dried. Alternatively, in the application of the couplers as alkali-soluble couplers, a coupler is dissolved in an aqueous solution of a caustic alkali, alkali carbonate, etc. or in an aqueous alcohol solution. Addition of the coupler to a silver halide emulsion may be made after or before the pH adjustment of the coupler-alkali solution with an aqueous citric acid solution. The treated emulsion is then coated on a support and dried.

Addition of the coupler to a silver halide emulsion may be made according to a known method in a preferable amount of 15-100 g. per mol of the silver halide contained in said emulsion. The amount added is, however, variable in the present invention.

The light-sensitive color photographic material thus prepared is exposed to light and treated according to an ordinary developing treatment. Dye image obtainable from such color photographic material is improved in transparency and has desirable spectral absorption characteristics. Further, crystallization of coupler out of the emulsion is remarkably inhibited, light scattering is not caused and unexposed area is also improved in transparency.

Typical developing solutions used in this invention contain in the form of sulfates, sulfites or hydrochlorides the following developing agents:

- 15 N,N-diethyl-p-phenylenediamine  
 N-ethyl-N- $\beta$ -methanesulfonamidoethyl-2-methyl-p-phenylenediamine  
 N-ethyl-N-hydroxyethyl-2-methyl-p-phenylenediamine  
 N-ethyl-N-hydroxyethyl-p-phenylenediamine  
 20 N,N-diethyl-2-methyl-p-phenylenediamine  
 25 N,N-diethyl-2-methyl-p-phenylenediamine

Melting points of  $\alpha$ -alkoxycarbonyl fatty acid amide coupler used in this invention and a known coupler having closely related structure to that of the above coupler are 30 compared in Tables 1 and 2 below.

TABLE 1  
 Comparison in melting point between the Coupler No. (2) and a known coupler similar thereto in structure

| Coupler                                    | Structural formula | M.P. (° C.) |
|--------------------------------------------|--------------------|-------------|
| Coupler (No. 2)-----                       |                    | 67-69       |
| Coupler disclosed in U.S.P. 2,875,057----- |                    | 126-127     |

TABLE 2  
 Comparison in melting point between the Coupler No. (9) and a known coupler similar thereto in structure

| Coupler                                    | Structural formula | M.P. (° C.) |
|--------------------------------------------|--------------------|-------------|
| Coupler No. (9)-----                       |                    | 48-49       |
| Coupler disclosed in U.S.P. 2,618,641----- |                    | 138-139     |

## 11

As evident from the above tables, melting points of the couplers used in this invention are extremely lower than those of the known couplers and therefore crystallization out of the emulsion or coating is inhibited. Thus, stabilized light-sensitive photographic material is made according to this invention.

Solubility of couplers used in this invention in a high boiling solvent is compared with that of known couplers having closely related structural formulas to those of the above couplers. Comparison is made by measuring a temperature at which 1.0 g. of a coupler dissolves in 2.0 ml. of dibutyl phthalate and an amount (ml.) of dibutyl phthalate required for dissolving 1.0 g. of a coupler at 45° C.

## 12

increase color density and are advantageously used in a reduced amount. The light-sensitive photographic material according to this invention has photographic properties improved in color reproduction and graininess.

5 Further, solubility of the  $\alpha$ -carboxy fatty acid amide type coupler used in the present invention in an aqueous alkali solution is compared with that of a known coupler having closely related structural formula to that of the

10 above coupler.

For comparison, a solution of 1.0 g. of coupler 5.0 ml. of N-potassium hydroxide aqueous solution is diluted with water to 100 ml. and  $\frac{1}{10}$  N-citric acid aqueous solution

TABLE 3  
Comparison in solubility between the Coupler No. (2) and a known coupler similar thereto in structure

| Coupler                                    | Structural formula | Temperature (° C.) | Amount of dibutyl phthalate (ml.) |
|--------------------------------------------|--------------------|--------------------|-----------------------------------|
| Coupler No. (2)-----                       |                    | 43                 | 2.0                               |
| Coupler disclosed in U.S.P. 2,875,057----- |                    | 80                 | 15.0                              |

TABLE 4  
Comparison in solubility between the Coupler No. (9) and a known coupler similar thereto in structure

| Coupler                                    | Structural formula | Temperature (° C.) | Amount of dibutyl phthalate (ml.) |
|--------------------------------------------|--------------------|--------------------|-----------------------------------|
| Coupler No. (9)-----                       |                    | 40                 | 1.5                               |
| Coupler disclosed in U.S.P. 2,618,641----- |                    | 50                 | 2.0                               |

As obvious from the above test results, the couplers used in this invention are superior in the solubility in a high boiling solvent to the known couplers and therefore useful also as protected couplers. Moreover, the couplers

is dropped with stirring at  $22 \pm 1^\circ$  C. until a turbid solution is formed with separation of precipitate. The pH value of the resulting solution is measured (pH at crystallization).

## 13

TABLE 5

Comparison in solubility between the Coupler No. (6) and a known coupler similar thereto in structure

| Coupler                                                 | Structural formula | pH at crystallization |
|---------------------------------------------------------|--------------------|-----------------------|
| Coupler No. (6) ---                                     |                    | 5.0                   |
| Coupler disclosed in Japanese Pat. Publn. No. 12836/66. |                    | 6.8                   |

TABLE 6  
Comparison in solubility between the Coupler No. (3) and a known coupler similar thereto in structure

| Coupler                                                    | Structural formula | pH at crystallization |
|------------------------------------------------------------|--------------------|-----------------------|
| Coupler No. (3) ---                                        |                    | 5.5                   |
| Coupler disclosed in Japanese Pat. Publn. No. 18735/64 --- |                    | 6.6                   |

As obvious from the above test results, the couplers used in the present invention are superior also in the solubility in an aqueous alkali solution to the known couplers and therefore very useful as alkali-soluble couplers. Like as in the application as protected couplers, the couplers used in the present invention are free from crystallization out of the emulsion or coating in the application as alkali-soluble couplers. Moreover, the couplers increase color density and are satisfactorily usable in a reduced amount. Besides, the light-sensitive photographic material according to the present invention has photographic properties improved in color reproduction and graininess.

In order that the present invention may be well understood, the following examples are given by way of illustration only.

## EXAMPLE 1

20 g. of the coupler No. (1) are dissolved in the mixture comprising 20 ml. of dibutyl phthalate and 60 ml. of butyl acetate at 80° C. Mixture of the resulting solution with 10 ml. of 10% aqueous solution of Alkanol B (alkyl-naphthalenesulfonate of Du Pont) and 200 ml. of 5% aqueous gelatin solution is passed through a colloid mill.

The dispersion obtained is added to 1 kg. of a high speed gelatino silver bromoiodide emulsion. The thus treated emulsion is coated on a film base and dried. The resulting light-sensitive photographic material is then exposed to light in an ordinary manner and treated at 20° C. for 10 minutes with a developing solution having the following formulation:

|                                              | G.   |
|----------------------------------------------|------|
| N,N-diethyl-p-phenylenediamine hydrochloride | 2.5  |
| Sodium sulfite (anhydrous)                   | 2.0  |
| Sodium carbonate (monohydrate)               | 82.0 |
| Potassium bromide                            | 2.0  |
| Water to make up to 1000 ml.                 |      |

Whereafter, the photographic material is subjected to ordinary stopping, fixing and water washing for 10-15 minutes, and treated for 5 minutes with a bleaching solution having the following formulation:

|                              | G.  |
|------------------------------|-----|
| Potassium ferricyanide       | 100 |
| Potassium bromide            | 50  |
| Water to make up to 1000 ml. |     |

After water washing for 5 minutes, the photographic material is treated for 5 minutes in the fixing bath comprising

|                                   | G.  |
|-----------------------------------|-----|
| Sodium thiosulfate (pentahydrate) | 250 |
| Water to make up to 1000 ml.      |     |

The light-sensitive photographic material thus treated is washed with water for 20-25 minutes and dried. Clear yellow dye image improved in spectral absorption characteristic and having the maximum absorption at 440 m $\mu$  is obtained.

A light-sensitive photographic material wherein the coupler No. (9) is dispersed in the emulsion in the same manner as above provides magenta dye image improved in spectral absorption characteristic and having the maximum absorption at 540 m $\mu$ , after light-exposure and subsequent color development effected in the same manner as above.

## EXAMPLE 2

10 g. of the coupler No. (2) are dissolved in the mixture comprising 10 ml. of tricresyl phosphate and 30 ml. of butyl acetate at 60° C. Mixture of the resulting solution with 5 ml. of 10% aqueous solution of Alkanol B and 200 ml. of 5% aqueous gelatin solution is passed through a colloid mill.

The dispersion obtained is added to 500 g. of a gelatino silver bromoiodide emulsion. The thus treated emulsion is coated on a film base and dried. The resulting light-sensitive photographic material is then exposed to light and treated at 20° C. for 10 minutes with a developing solution having the following formulation:

|                              | G.   |
|------------------------------|------|
| Metol                        | 3.0  |
| Sodium sulfite (anhydrous)   | 60.0 |
| Hydroquinone                 | 6.0  |
| Sodium carbonate (anhydrous) | 50.0 |
| Potassium bromide            | 1.0  |
| Water to make up to 1000 ml. |      |

## 15

After being subjected to ordinary stopping, hardening and water washing treatments, the photographic material is re-exposed to white light and treated at 20° C. for 12 minutes with a developing solution having the following formulation:

|                                              |      |
|----------------------------------------------|------|
|                                              | G.   |
| N,N-diethyl-p-phenylenediamine hydrochloride | 5.0  |
| Sodium sulfite (anhydrous)                   | 2.0  |
| Sodium carbonate (monohydrate)               | 82.0 |
| Potassium bromide                            | 1.0  |
| Water to make up to 1000 ml.                 |      |

Whereafter, the stopping, fixing, water washing and bleaching treatments are effected in a usual manner and the thus treated light-sensitive photographic material is washed with running water for 20 minutes and dried. Yellow positive dye image improved in transparency and having the maximum absorption at 445 m $\mu$  is obtained.

A light-sensitive photographic material wherein the coupler No. (11) is dispersed in the emulsion in the same manner as above provides clear magenta dye image improved in transparency and having the maximum absorption at 535 m $\mu$ .

## EXAMPLE 3

10 g. of the coupler No. (6) are dissolved in 20 ml. of dibutyl phthalate at 50° C. Mixture of the resulting solution with 5 ml. of 10% aqueous solution of Alkanol B and 200 ml. of 5% aqueous gelatin solution is passed through a colloid mill several times. The resulting dispersion is added to 500 g. of a gelatino silver chlorobromide emulsion. The treated emulsion is coated on a baryta paper and dried.

The resulting light-sensitive photographic material is then exposed to light and treated at 20° C. for 10 minutes with a developing solution having the following formulation:

|                                                             |      |
|-------------------------------------------------------------|------|
|                                                             | G.   |
| N - ethyl - N - hydroxyethyl - p - phenylenediamine sulfate | 2.5  |
| Sodium sulfite (anhydrous)                                  | 2.0  |
| Hydroxylamine hydrochloride                                 | 1.0  |
| Sodium carbonate (monohydrate)                              | 82.0 |
| Potassium bromide                                           | 2.0  |
| Water to make up to 1000 ml.                                |      |

Subsequently, stopping is effected in the stopping bath comprising 10 ml. of glacial acetic acid, 3.0 g. of sodium hydroxide and 1000 ml. of water and immediately thereafter fixing is effected for 4 minutes in an acidic fixing solution. After washing with water for 10 minutes, the photographic material is treated at 20° C. for 8 minutes with a bleaching solution having the following formulation:

|                                      |       |
|--------------------------------------|-------|
|                                      | G.    |
| Disodium ethylenediaminetetraacetate | 40.0  |
| Ferric chloride                      | 30.0  |
| Sodium carbonate (monohydrate)       | 20.0  |
| Potassium bromide                    | 30.0  |
| Sodium thiosulfate (pentahydrate)    | 200.0 |
| Water to make up to 1000 ml.         |       |

The photographic material thus treated is subjected to water washing for 20 minutes and stabilizing for 2 minutes and then dried. Thus, magenta dye image having the maximum absorption at 535 m $\mu$  and improved in fastness to light, heat and humidity is obtained.

## EXAMPLE 4

A solution of 10.0 g. of the coupler No. (8) in 60 ml. of N-potassium hydroxide aqueous solution is diluted with water to 200 ml. and adjusted with N-citric acid aqueous solution to pH 6.8. The resulting solution is added to 1 kg. of high speed gelatino silver bromoiodide emulsion. The treated emulsion is coated on a film base and dried. The resulting light-sensitive photographic material is then ex-

## 16

posed to light and treated at 20° C. for 10 minutes with a developing solution having the following formulation:

|                                             |      |
|---------------------------------------------|------|
|                                             | G.   |
| N,N-diethylamino-p-phenylenediamine sulfate | 2.5  |
| Sodium sulfite (anhydrous)                  | 2.0  |
| Sodium carbonate (monohydrate)              | 82.0 |
| Potassium bromide                           | 2.0  |
| Water to make up to 1000 ml.                |      |

Being subjected to stopping and fixing in a usual manner, the photographic material thus treated is washed with water for 10-15 minutes and then treated for 5 minutes with a bleaching solution having the following formulation:

|                        |       |
|------------------------|-------|
|                        | G.    |
| Potassium ferricyanide | 100.0 |
| Potassium bromide      | 50.0  |

Water to make up to 1000 ml. The resulting film is further washed with water for 10 minutes and fixed for 5 minutes in the fixing bath comprising

|                    |     |
|--------------------|-----|
|                    | G.  |
| Sodium thiosulfate | 250 |

Water to make up to 1000 ml. After water washing and drying the film, magenta dye image having the maximum absorption at 535 m $\mu$  and improved in transparency is obtained.

From a light-sensitive photographic material wherein the coupler No. (3) is dispersed in the emulsion and the same treatments as above are effected, is obtained clear yellow dye image having the maximum absorption at 440 m $\mu$ .

## EXAMPLE 5

A mixture of 10.0 g. of the coupler No. (9) and 30 ml. of ethanol is dissolved in 10 ml. of 20% potassium hydroxide aqueous solution at 60° C. The resulting solution is diluted with water to 200 ml. and pH value is adjusted. This solution is added to 1 kg. of high speed gelatino silver bromoiodide emulsion and the resulting emulsion is coated on a support and dried.

The light-sensitive photographic material thus obtained is subjected to light-exposure and color development under the same conditions described in the Example 4. Thus, clear magenta dye image having the maximum absorption at 537 m $\mu$  is obtained.

What is claimed is:

1. A light-sensitive color photographic silver halide emulsion which comprises a coupler of the general formula



wherein

R represents a radical which couples with the oxidation 8-20 carbon atoms,

R<sub>2</sub> represents hydrogen or a lower alkyl group,

B represents a radical which couples with the oxidation product formed during color development to form a yellow or magenta color,

X represents a radical connecting B and



n is 0 or 1.

2. A light-sensitive color photographic silver halide emulsion as claimed in the claim 1, wherein a coupler of the general formula is the compound of the following formula



3. A light-sensitive color photographic silver halide emulsion as claimed in the claim 1, wherein a coupler

17

of the general formula is the compound of the following formula



4. A light-sensitive color photographic silver halide emulsion as claimed in the claim 1, wherein a coupler of 10 the general formula is the compound of the following formula



5. A light-sensitive color photographic silver halide emulsion as claimed in the claim 1, wherein a coupler 30 96-55

18

of the general formula is the compound of the following formula



15 6. An emulsion according to claim 1 wherein X is a phenylene group.  
7. An emulsion according to claim 6 wherein X is p-phenylene or n-phenylene.

20

#### References Cited

##### UNITED STATES PATENTS

2,875,057 2/1959 McCrossen et al. ----- 96-100  
2,829,975 4/1958 Popeck et al. ----- 96-55

25 NORMAN G. TORCHIN, Primary Examiner  
E. C. KIMLIN, Assistant Examiner

U.S. Cl. X.R.